

## UNITED STATES PATENT OFFICE

2,257,869

## INSULATING OIL COMPOSITIONS

Charles E. Trautman, East McKeesport, Pa., assignor to Gulf Research & Development Company, Pittsburgh, Pa., a corporation of Delaware

No Drawing. Application March 22, 1940,  
Serial No. 325,479

4 Claims. (Cl. 252—63)

This invention or discovery relates to insulating oil compositions; and it comprises such a composition, particularly a transformer oil, highly resistant to deterioration by oxidation and including a petroleum oil containing a small amount of an aniline derivative selected from the class consisting of benzyl-p-anisidine and benzyl-p-phenetidine; all as more fully herein-after set forth and as claimed.

In many types of electrical transformers the core and windings are immersed in a suitable petroleum oil, for serving as a dielectric and for carrying heat away from the core and windings. The requirements of a transformer oil include good dielectric properties, low viscosity to facilitate heat transfer for convection, low pour point to avoid solidification of the oil by cold, high flash and fire points to minimize danger of fire and explosion and low volatility to reduce evaporation losses. In addition the oil must be resistant to oxidation, and must be of such character as to resist emulsification with water.

Transformer oils ordinarily are distillate oils refined in such manner as to secure the specified characteristics to as great an extent as possible. Achievement of satisfactory oxidation resistance is difficult, for while oxidation changes are slow, transformer oils are ordinarily expected to remain in service over long periods. Oxidational changes result in the formation of insoluble matter or sludge. The sludge tends to render the oil more miscible with water, with production of emulsions in the presence of condensed water and a consequent degradation of the dielectric properties of the oil body. The sludge also deposits on the windings and core with reduction of the efficiency of heat transfer. Oxidation of transformer oils tends to be promoted by contact with metals, especially copper, and with the usual varnishes and insulating materials.

Various materials have been proposed for incorporation into transformer oils with the object of inhibiting oxidation, and some of these have come into use. The usual anti-oxidants may be divided in two principle classes: (1) those which are associated with a lengthening of the induction period, that is the time which elapses before appearance of sludge in the oil subject to oxidation, and (2) those which reduce the amount of sludge formed per day after it once begins to form. In evaluating oils containing anti-oxidants, the most useful criterion is a value which takes into account both these characteristics, viz., the time required, under the test conditions,

to form a definite amount of sludge, say 0.1 per cent by weight of the oil.

I have discovered an anti-oxidant which brings about both a marked lengthening of the induction period and a lessening of the rate of sludge formation, when incorporated in transformer oils even in minimal amounts. The anti-oxidant has certain other advantages. It is quite soluble in oil, more so than many other anti-oxidants, but is highly insoluble in water, thereby minimizing the tendency to formation of aqueous emulsions. In the best embodiment of the invention the anti-oxidant is a compound which can be represented by the structural formula



and may be termed benzyl-p-anisidine or N-benzyl-4-methoxyaniline. The methoxy group (OCH<sub>3</sub>) can be replaced by an ethoxy group (OC<sub>2</sub>H<sub>5</sub>); such compound, benzyl-p-phenetidine or N-benzyl-4-ethoxyaniline, gives somewhat similar results. These compounds when added to transformer oils and other electrical insulating oils in amounts corresponding to about 0.05 to 0.5 per cent by weight of the oil effectively stabilize such oils against oxidation deterioration.

My anti-oxidant can be employed if desired in conjunction with other anti-oxidants but it is so effective, both as regards prolonging the induction period and minimizing the rate of sludge formation, as to render addition of other types of anti-oxidants unnecessary. When very small proportions of my antioxidant are used in the oil, it is sometimes convenient to incorporate a little of certain alkylation products of phenols and substituted phenols in which there are present alkylation linkages of secondary or tertiary type, and exemplified by the compounds;

- 2,6-di-tertiary-butyl-4-methyl phenol
- 2,6-di-tertiary-butyl-4-ethyl phenol
- 2,6-di-tertiary-butyl-4-cyclohexyl phenol
- 2,6-di-tertiary-butyl-4-benzyl phenol
- 2,4,6-tri-tertiary-butyl phenol
- 2,6-di-tertiary-amyl-4-methyl phenol

In the following table, comparative oxidation test results are set forth for oils containing the new anti-oxidant, for an untreated oil, and for certain other anti-oxidants not part of the invention. The test data were obtained in accordance with the sludge formation test for mineral transformer oil, described by F. M. Clark and E. A. Snyder in their paper entitled "Test-

ing for Sludge Formation in Mineral Transformer Oil" presented at the Thirty-ninth Annual Meeting for the American Society for Testing Materials. The test procedure described in the aforesaid paper was developed in collaboration with the laboratories of a considerable number of firms engaged in oil refining and in the manufacture of electrical equipment.

In this test, samples of oil are maintained in tubes containing copper wire at a constant temperature of approximately 120° C. The tubes are open at the top to an enclosed air space and dry air is passed at a controlled rate of 1½ to 2 cubic feet per hour through the enclosed space above the sample tubes. Into each tube is introduced 22 grams of oil or oil composition to be tested, a number of tubes being employed. At prescribed intervals the tubes are successively removed and the amount of sludge determined. The results of these tests are reported in terms of the induction period, the per cent of sludge formed per day and the total number of days taken to form 0.1 per cent of sludge.

The oil employed in all of the tests set forth hereinbelow was a typical petroleum transformer oil, commonly used for the purpose indicated.

*Transformer oil sludge formation test carried out at 120° C. in the presence of copper*

| Test No. | Inhibitor                                                               | Induction period | Rate of sludge formation, in 0.01% per day, after induction period | Time to form 0.1% sludge |
|----------|-------------------------------------------------------------------------|------------------|--------------------------------------------------------------------|--------------------------|
| 1.       | None                                                                    | Days 0           | 1.13                                                               | 7                        |
| 2.       | Benzyl-p-anisidine 0.1%                                                 | 3                | 0.75                                                               | 17                       |
| 3.       | Ditto 0.3%                                                              | 5                | 0.18                                                               | 60 or more               |
| 4.       | Ditto 0.5%                                                              | 5                | 0.18                                                               | 60 or more               |
| 5.       | Ditto 0.1% plus 2,6-di-tertiary-butyl-4-methyl phenol 0.3%              | 5                | 0.18                                                               | 60 or more               |
| 6.       | Benzyl-p-anisidine 0.3% plus 2,6-di-tertiary-butyl-4-methyl phenol 0.3% | 5                | 0.18                                                               | 60 or more               |
| 7.       | 2,6-di-tertiary-butyl-4-methyl phenol 0.3%                              | 10               | 2.40                                                               | 14                       |
| 8.       | Monobenzyl-p-aminophenol (sat'd) 0.03%                                  | 0                | 0.35                                                               | 28                       |
| 9.       | Dibenzyl-p-anisidine 0.3%                                               | 1                | 1.18                                                               | 5                        |
| 10.      | Acetyl-p-anisidine, saturated (less than 0.3%)                          | 0                | 1.25                                                               | 5                        |
| 11.      | p-Anisidine 0.3%                                                        | 0                | 1.25                                                               | 6                        |
| 12.      | p-Phenetidine 0.3%                                                      | 0                | 4.00                                                               | 3                        |
| 13.      | Benzyl aniline 0.3%                                                     | 2                | 1.00                                                               | 11                       |

In the table, tests 1 to 6 relate to composi-

55

CHARLES E. TRAUTMAN.

CERTIFICATE OF CORRECTION.

Patent No. 2,257,869.

CHARLES E. TRAUTMAN.

October 7, 1941.

It is hereby certified that error appears in the printed specification of the above numbered patent requiring correction as follows: Page 2, second column, line 48, claim 3, for "0.5 to 0.5" read --0.05 to 0.5--; and that the said Letters Patent should be read with this correction therein that the same may conform to the record of the case in the Patent Office.

Signed and sealed this 11th day of November, A. D. 1941.

Henry Van Arsdale,  
Acting Commissioner of Patents.

(Seal)

CERTIFICATE OF CORRECTION.

Patent No. 2,257,869.

October 7, 1941.

CHARLES E. TRAUTMAN.

It is hereby certified that error appears in the printed specification of the above numbered patent requiring correction as follows: Page 2, second column, line 48, claim 3, for "0.5 to 0.5" read --0.05 to 0.5--; and that the said Letters Patent should be read with this correction therein that the same may conform to the record of the case in the Patent Office.

Signed and sealed this 11th day of November, A. D. 1941.

Henry Van Arsdale,  
Acting Commissioner of Patents.

(Seal)